

June 3, 1958

K. J. DE VOS ET AL

2,837,452

METHOD OF MAKING ANISOTROPIC PERMANENT MAGNETS

Filed Jan. 18, 1956



KRIJN JACOBUS DE VOS  
ADOLF JOHANNES JACOBUS KOCH  
HENDRIK JOHANNES MEERKAMP VAN EMBDEN  
BARTHOLOMEUS HAES  
JOHANNES FLIPSE

BY

*De Vos*  
AGENT

1

2,837,452

METHOD OF MAKING ANISOTROPIC  
PERMANENT MAGNETS

Krijn Jacobus de Vos, Adolf Johannus Jacobus Koch, Hendrik Johannes Meerkamp Van Embden, Bartholomeus Haes, and Johannes Flipse, Eindhoven, Netherlands, assignors, by mesne assignments, to North American Philips Company, Inc., New York, N. Y., a corporation of Delaware

Application January 18, 1956, Serial No. 559,982

Claims priority, application Netherlands January 19, 1955

5 Claims. (Cl. 148—103)

Methods are known for making anisotropic permanent magnets containing up to 42% of Co, 10% to 20% of Ni, 6% to 10% of Al, 2% to 8% of Cu, 4% to 10% of Ti and Fe, in order to secure a high coercivity ( $B_H$ )<sub>c</sub> of more than 900 oersteds and a high ( $BH$ )<sub>max</sub> value, the alloys being cooled from a temperature of approximately 1225° C. to a temperature of 600° C. in a magnetic field at an average cooling rate of at least 30° C./min. to 600° C./min. With several of such magnets the coercivity is 1080 oersteds with a ( $BH$ )<sub>max</sub> value of 2,460,000 g. oersteds, 1140 oersteds with 3,500,000 g. oersteds and 925 oersteds with 4,100,000 g. oersteds respectively. Such magnets have the advantage that they can be used in constructions wherein strong demagnetizing fields prevail. This means that the magnet may have a very small length.

The present invention is based on the discovery that the aforesaid magnets, when subjected to a particular heat-treatment while retaining a high coercivity in excess of 900 oersteds and in the majority of cases even with an increase in coercivity, reach a considerably higher ( $BH$ )<sub>max</sub> value.

In accordance with our invention, the aforesaid alloy, which contains 15% to 42% of Co, after being quenched from a temperature higher than about 1200° C. to at least about 900° C. is maintained, under the action of a magnetic field, in a temperature range of from about 10° to 70° C. below the Curie-temperature for 2 to 30 minutes, preferably for at least 4 to 15 minutes at a substantially constant temperature, varying less than 20° C. In this manner a magnet is obtained having a ( $BH$ )<sub>max</sub> value exceeding at least 700,000 g. oersteds the ( $BH$ )<sub>max</sub> value

2

of a magnet obtained by the usual cooling of at least 30° C./min. in said temperature range.

The aforesaid substantially constant temperature is obtainable by subjecting the alloys to the action of the magnetic field, in a metal or salt bath of suitable temperature or in an oven. In practice, said temperature variation of less than 20° C. may occur in ovens since the temperature of these cannot be maintained at a strictly constant level.

10 The alloy, after being quenched to a temperature of 900° C., may be further cooled to room temperature and subsequently heated into the desired temperature range below the Curie-temperature for treatment in a magnetic field. Alternatively, the alloy may be cooled rapidly from 900° C. into the desired temperature range.

15 After treatment in a magnetic field, cooling to room temperature may be effected by any convenient means, provided it is not done too slowly. A normal annealing treatment may then follow this treatment.

20 This invention permits the manufacture of magnets in which said improvement of the ( $BH$ )<sub>max</sub> value is at least 1,000,000 g. oersteds.

25 The process of our invention is of particular advantage when applied to alloys containing more than 30% to 42% of Co.

30 Should a predominating crystal orientation be desired, in order to secure better magnetic properties, the melt may be caused to solidify directionally by cooling slowly, for example in an oven, in accordance with Dutch Patent Specification 71,925.

35 In the following tables several examples are given stating the time periods during which the alloys stayed in the temperature range of 10° C. to 70° C. below the Curie-temperature, the following heat treatment being employed:

40 After solidification, the alloys were quenched in compressed air. From room temperature they were reheated to the temperature listed in the tables and maintained on said temperature for the stated number of minutes. Subsequently, they were cooled and annealed at an average cooling rate of approximately 2° C./sec.

45 The first line states for each alloy the  $B_r$ , the  $H_c$  and the  $(BH)_{max} \times 10^{-6}$  respectively for a magnet of the same composition but cooled from more than 1200° C. to about 600° C. at a rate of about 30 to 60° C./min.

Table

| Co | Ni   | Al  | Cu  | Ti | Curie temperature in 0° C. | Hardening temperature in 0° C. | Min. | $B_r$ | $H_c$ | $(BH)_{max} \times 10^{-6}$ | Profit of $(BH)_{max} \times 10^{-6}$ |
|----|------|-----|-----|----|----------------------------|--------------------------------|------|-------|-------|-----------------------------|---------------------------------------|
| 18 | 20   | 7   | 6   | 5  | 835                        | 780                            | 3    | 6,840 | 870   | 1.65                        | 1.                                    |
|    |      |     |     |    |                            | 800                            | 2    | 7,420 | 922   | 2.6                         |                                       |
|    |      |     |     |    |                            | 815                            | 2    | 7,580 | 960   | 2.8                         |                                       |
| 24 | 14   | 8   | 3   | 5  | 865                        | 825                            | 9    | 7,560 | 950   | 2.7                         | 0.8                                   |
|    |      |     |     |    |                            | 825                            | 9    | 7,820 | 740   | 2.55                        |                                       |
|    |      |     |     |    |                            | 825                            | 9    | 8,280 | 950   | 3.35                        |                                       |
| 30 | 14   | 7.5 | 3.5 | 5  | 840                        | 800                            | 9    | 9,020 | 946   | 3.7                         | 0.7-1.0                               |
|    |      |     |     |    |                            | 800                            | 15   | 9,100 | 1,150 | 4.4                         |                                       |
|    |      |     |     |    |                            | 815                            | 5    | 9,320 | 1,150 | 4.5                         |                                       |
| 34 | 14.5 | 7   | 4.5 | 5  | 845                        | 815                            | 9    | 9,200 | 1,180 | 4.4                         | 0.8-1.3                               |
|    |      |     |     |    |                            | 780                            | 20   | 9,000 | 1,220 | 4.7                         |                                       |
|    |      |     |     |    |                            | 790                            | 4    | 9,200 | 1,200 | 4.6                         |                                       |
| 40 | 14.5 | 7   | 4.5 | 5  | 855                        | 790                            | 6    | 9,200 | 1,260 | 4.8                         | 1.1-1.2                               |
|    |      |     |     |    |                            | 790                            | 8    | 9,100 | 1,300 | 4.9                         |                                       |
|    |      |     |     |    |                            | 790                            | 13   | 9,200 | 1,200 | 4.7                         |                                       |
| 40 | 14.5 | 7   | 4.5 | 5  | 855                        | 800                            | 20   | 9,250 | 1,175 | 4.65                        | 1.4                                   |
|    |      |     |     |    |                            | 800                            | 2    | 9,200 | 1,260 | 4.6                         |                                       |
|    |      |     |     |    |                            | 800                            | 6    | 9,200 | 1,290 | 4.8                         |                                       |
| 40 | 14.5 | 7   | 4.5 | 8  | 815                        | 800                            | 8    | 9,300 | 1,300 | 4.95                        | 1.4                                   |
|    |      |     |     |    |                            | 800                            | 13   | 9,550 | 1,300 | 5.1                         |                                       |
|    |      |     |     |    |                            | 800                            | 3    | 8,800 | 950   | 3.0                         |                                       |
| 40 | 14.5 | 7   | 4.5 | 8  | 815                        | 800                            | 8    | 9,020 | 1,160 | 4.2                         | 1.4                                   |
|    |      |     |     |    |                            | 800                            | 3    | 8,880 | 1,230 | 4.15                        |                                       |
|    |      |     |     |    |                            | 810                            | 3    | 8,980 | 1,150 | 4.1                         |                                       |
| 40 | 14.5 | 7   | 4.5 | 8  | 815                        | 810                            | 3    | 6,100 | 1,046 | 1.65                        | 1.4                                   |
|    |      |     |     |    |                            | 815                            | 5    | 6,860 | 1,400 | 3.05                        |                                       |
|    |      |     |     |    |                            | 815                            | 5    | 6,900 | 1,400 | 3.05                        |                                       |

Two examples are now given of magnets having a preponderating crystal orientation. In this case directional solidification of the melt ensued by slow cooling of the liquid alloy in an oven having a temperature of 1500° C. till the alloy has solidified, the alloys subsequently being reheated and treated in the aforesaid manner.

| Co       | Ni         | Al       | Cu         | Ti     | ° C.       | Min.    | B <sub>r</sub>  | H <sub>o</sub> | (BH) <sub>max</sub> × 10 <sup>-3</sup> |
|----------|------------|----------|------------|--------|------------|---------|-----------------|----------------|----------------------------------------|
| 30<br>34 | 14<br>14.5 | 7.5<br>7 | 3.5<br>4.5 | 5<br>5 | 800<br>800 | 10<br>8 | 9,800<br>10,000 | 1,310<br>1,580 | 5.8<br>7.5                             |

The accompanying diagram shows the (BH)<sub>max</sub> value in accordance with the Co value for magnets of the same composition with 5% of Ti, the upper curve concerning alloys treated in accordance with the invention and the lower curve relating to alloys treated in accordance with the usual method, the improvement upon the (BH)<sub>max</sub> value being clearly evidenced.

While we have described our invention in connection with specific embodiments and applications, other modifications thereof will be readily apparent to those skilled in this art without departing from the spirit and scope of the invention as defined in the appended claims.

What is claimed is:

1. In the manufacture of a permanent magnet, the steps of forming a body of a ferrous alloy containing about 15 to 42% cobalt, about 10 to 20% nickel, about 6 to 10% aluminium, about 2 to 8% copper, about 4 to 10% titanium and the balance principally iron, quenching said body from a temperature exceeding about 1200° C. to a temperature of about 900° C., and subjecting said body to the action of a magnetic field while said body is maintained at a substantially constant temperature varying less than about 20° C. in a range of about 10° to 70°

5 C. below its Curie temperature for about 2 to 30 minutes whereby an anisotropic permanent magnet having a substantially increased (BH)<sub>max</sub> is obtained.

2. In the manufacture of a permanent magnet, the steps of forming a body of a ferrous alloy containing about 15 to 42% cobalt, about 10 to 20% nickel, about

15 6 to 10% aluminium, about 2 to 8% copper, about 4 to 10% titanium and the balance principally iron, quenching said body from a temperature exceeding about 1200° C. to a temperature of about 900° C., and subjecting said body to the action of a magnetic field while said body is maintained at a substantially constant temperature varying less than about 20° C. in a range of about 10° to 70° C. below its Curie temperature for about 4 to 15 minutes whereby an anisotropic permanent magnet having a substantially increased (BH)<sub>max</sub> is obtained.

20 3. The process of claim 1 in which the alloy contains from more than 30% to 42% of Co.

25 4. The method of claim 1 in which the alloy is slowly caused to solidify to cause a predominant crystal orientation before being subjected to the magnetic field and constant temperature treatment.

30 5. A permanent magnet made by the process of claim 1.

#### References Cited in the file of this patent

#### UNITED STATES PATENTS

35 2,499,860 Hansen ----- Mar. 7, 1950  
2,578,407 Ebeling ----- Dec. 11, 1951